

June 12, 1934.

E. R. POWELL

1,963,031

CELLULAR CERAMIC PROCESS AND APPARATUS



Fig. 2.



June 12, 1934.

E. R. POWELL

1,963,031

CELLULAR CERAMIC PROCESS AND APPARATUS

Original Filed March 29, 1932 2 Sheets-Sheet 2



INVENTOR.

*Edward R. Powell.*

## UNITED STATES PATENT OFFICE

1,963,031

## CELLULAR-CERAMIC PROCESS AND APPARATUS

Edward R. Powell, Alexandria, Ind.

Application March 29, 1932, Serial No. 601,796  
Renewed January 30, 1934

11 Claims. (Cl. 25—1)

This invention relates to a cellular ceramic material.

It relates particularly to a ceramic building material in which there are air cells or air spaces, 5 the solid material or ceramic material proper comprising an expanded or cellular structure which encloses or nearly encloses these air cells. This structure results from the principal features of the invention which comprise the formation of gas bubbles within the material while it is in wet liquid condition and the subsequent preservation of the bubbled or expanded stock thus formed until the material is finally dried and fired to the hard or vitrified condition which 10 is characteristic of ceramic ware; such drying being of a character that it does not materially 15 destroy the expanded structure previously imparted thereto.

The advantages of a material of this type over 20 solid brick or tile are: (1) Low shipping and handling weights which permit larger units and lighter foundations and framework. (2) Higher 25 thermal resistance so that, when the material is built into walls, better heat barriers will be formed. (3) Adaptability such as easier drilling and cutting and anchoring of screws and nails. (4) Better bonding of mortars on unglazed faces due to the open structure which permits the mortar to enter and bond. (5) Better acoustical 30 properties when the cells are of the proper type and the cellular arrangement is exposed.

The cellular material has a density of about 30 to 50 lbs. per cu. ft. as compared to 120 to 150 lbs. for solid ceramic material such as 35 commercial brick or solid tile. The other differences in properties are related to and result from these differences in density and structure.

The principal object of the invention is to 40 manufacture a material which has these advantages in a convenient and economical manner from any clay or shale which has fair plasticity when comminuted; and to do this without adding a large volume or percentage of combustible or volatile aggregate or setting reagents.

45 The chief feature of the invention consists in the accomplishment of this object by the use of certain processes and certain refinements of technique in the mixing of the clays and the relatively small amounts of chemicals so that a 50 desired amount and desired type of expansion are obtained; and in the subsequent molding, drying and burning to produce the desired product without material destruction of the cellular arrangement.

55 The process includes (1) the preparation of two

mutually chemically reactive supplies of liquid clay in free flowing condition but without any unnecessary proportion of water; (2) the mixing of these two liquid clays in order to free a gas and sometimes to produce other desirable results more specifically set forth hereinafter; the mixing being at such a rate that it is intimate and substantially complete before the major part of the reaction has taken place; (3) the delivering of this mixture with a minimum of disturbance to a drier; (4) the exposing in the drier of a relatively large surface of the material in proportion to the volume and depth thereof; (5) the hardening of this material by heating in expanded condition so that it will not readily remix 60 with water but is more or less water-absorbent; (6) the coating of the aggregate obtained from the last operation with more liquid reactive material as obtained from the second operation or other suitable binder to bond the material and 65 finally molding into shapes.

70 There are, naturally, numerous conventional operations both before, between and after the above operations. These include mining or winning of the clay, grinding, tempering, trimming, 75 separating into units, texturing, glazing, drying and burning. The invention, therefore, resides in the above mentioned operations, the apparatus therefor and the product therefrom taken in connection with the conventional processes practised in other ceramic art.

80 The full nature of the invention will be understood from the accompanying drawings and the following description and claims:

Fig. 1 is a flow sheet showing the passage of 85 the material through the process.

Fig. 2 is a diagrammatic layout of one form of apparatus suitable for practising the invention.

Fig. 3 is an enlarged plan of one form of continuous mixer, parts being shown in central section, said mixer being adapted to perform rapid continuous mixing.

Fig. 4 is an elevational view of another form of mixer for the same purpose as that of Fig. 3, 95 parts thereof being shown in central section.

Fig. 5 is a section through a structural unit of one form of finished product which is provided with an imperforate surface coating.

Fig. 6 is a similar view through another form 105 of finished product which is provided with a perforate coating.

Referring to Fig. 1, the two supplies of liquid clay 11 and 12 are withdrawn at 15 and 16 respectively and delivered to the fast mixing op- 110

eration at 17, the amount being regulated as at 13 and 14 respectively. The mixture is dried at 19, 20 and 21; is transferred at 22 to the heating operation at 23. A burning operation 5 at 24 supplies heat which is utilized in the heating operation at 23 and subsequently utilized in the drying operation and finally discharged at 38. The two supplies of liquid clay 26 and 27 are similarly withdrawn at 28 and 29, 30 and 31, 10 like 13 and 14, representing the step of feeding measured amounts of the clay. Heated aggregate 23 is measured and sized at 37—25. Liquid clays mixed at 32 are delivered at 33 and combined in the form of a coating on the aggregate 15 at 34. The coated or mixed material is withdrawn at 35 and passes to the molding operation at 36 where it is formed and sized to shape. The resulting mass is then dried, trimmed or separated into units if necessary and fired as in 20 other ceramic processes.

20 The preparation of the liquid clay may require more grinding than ordinarily practised in brick making. This extra grinding may be done wet or dry. The ground clay is mixed with water 25 and tempered to the right consistency.

25 A satisfactory formula for the clay in the liquid clay supply 11 may include 7 per cent finely powdered dolomite and 1 per cent soda ash based on the dry weight of the clay; and that for the 30 clay in the liquid clay supply 12 may include 2 per cent sulphuric acid, the extract from 1 per cent of soap bark and  $\frac{1}{4}$  per cent of karaya gum. The acid reacts with the dolomite and the soda ash to form carbon dioxide in the form of 35 bubbles. The soap bark has the effect of preserving the bubbles and the karaya gum stabilizes the froth temporarily.

40 The amount of clay from supply 12 may be less in proportion to that from supply 11. A clay of the colloidal type which is in deflocculated condition when acid is preferable for the material of clay supply 12. The liquid clays should both be initially in deflocculated condition so that a minimum of water is required to keep 45 them liquid, agitation of some sort often being required. The resulting mixture should preferably be flocculated, to hold the structure until dried. For this condition, the mixture should usually be nearly neutral or slightly acid. The 50 above example is for a carbonate-containing clay slip adapted to react with an acidulated clay slip. Other acids and carbonates may be used. Also other reactions such as caustic with zinc or aluminum dust may be employed.

55 The dried material usually crumbles easily and will break up in a rotary kiln to the desired size. If it is too large for the size slab to be molded, it may be crushed. It may be advisable to mold the material in large slabs, and separate into 60 smaller or thinner units while "green". For some purposes the ware may be molded to size and shape in a manner similar to wet mud brick making and need not be trimmed.

65 For minimum density in the completed product, the bonding material should preferably be expanded also, as represented by the fast mixing at 32.

70 For a "marble-ized" effect, the clays in the aggregate may "burn" to a different color from those of the bonding material. If the product is dressed or split and left uncoated, this effect will show in the finished product.

75 If desired, the reaction between the reactive liquid clays 11 and 12 or 26 and 27 may be so regulated (by their temperature and composi-

tion) that very little froth is formed until the mixture encounters the elevated temperature at 19—20—21; or at 34 where the mixture from 32 may encounter a hot or warm aggregate.

80 An example of apparatus suitable for practising the invention is shown in Figs. 2, 3 and 4. The clay supplies 11, 12, 26 and 27 may be in tanks of conventional type. They may require agitation by mechanical stirrers 66, or air agitation or circulation may be used. The pipes 15, 16, 28 and 29 should be large. As a safety measure, they 85 should be provided with water supplies for back washing to prevent clogging if the clay settles in the pipes. The above being standard practice, the apparatus is not shown. The feeding devices 14, 13, 30 and 31 may be gear pumps in which the clearances are larger than the particle size of the clay. Both impellers of the pumps should preferably be externally driven, so that 90 they will not contact in the presence of the clay. This avoids excessive wear if the clay is abrasive. It is advisable to have the speeds of these feeding devices controllable.

95 A satisfactory form of fast continuous mixer 100 17 and 32 is shown in Fig. 3. It consists of a motor 40 which drives a rotor 47 by means of a shaft 45. A casing 42 is sealed by a gland 43 and houses the rotor. The casing has passages 44 and 41 for admitting the supplies of liquid clay. The 105 clay is fed in by pressure and passes between the rotor and casing as the rotor revolves. The slightly conical passage 48 is small so that the clay passes through the mixer in a very short time. The speed of the rotor is such that the two 110 supplies are intimately mixed by the time they reach the outlet 46. The slight conical formation is for subsequent adjustment for wear and for adjustment according to the consistency of the material to be handled.

115 Another form of mixer is shown in Fig. 4. In this form, the two supplies of clay liquid are discharged at considerable velocity from two nozzles 50 and 51. They meet at 52 and form a mixed stream. To complete the mixing, the mingled 120 stream is deflected by inclined stationary vanes 54 and 55, which are opposite-disposed, and by forwardly inclined vane 53. By this method, the mixing is so rapid that the reaction is just starting when the material reaches the position 56. The reaction proceeds rapidly thereafter forming 125 the frothed condition indicated at position 57. The approximate enlargement resulting therefrom is indicated clearly in Fig. 4.

130 The clay flows from mixer 17 down chute 18 into conveyor 19. Ordinarily the clay is liquid enough to spread itself on the conveyor. If not, it may be spread by hand or mechanically to a thin layer or into small wads. The conveyor 19, oven 20, baffles 21 and chutes 18 and 22 may all 135 be of conventional type. Recirculation may be used in oven 20 to increase the air velocity. Kiln 23 and crusher 65 may be of conventional type. A commercial feeder 25 is provided as an outlet for bin 37. Fuel burner 24 indicates any convenient fuel burning apparatus. The fan in connection with the oil supply 67 forms an oil flame for generating heat. Powdered coal, gas or solid fuel may also be used. The tumbler type mixer 34 is similar to a concrete mixer, and includes a regular charging chute 33. The mixing may be 140 continuous or in batches. The molds 36 represent any form of mold desired. Removable forms on a turn table are often used for this service.

145 Fig. 5 represents a form of finished product which may be made by this process. For gen- 150

eral structural purposes, an imperforate washable coating 58 is desirable and the cells 61 in the aggregate and cells 60 in the binding medium are mainly self-contained or separate individual bubbles enclosed in walls of ceramic material. This structure is desirable for strength.

Fig. 6 represents another form of product in which the structure is very open, having reentrant cells 63 and 64, cracks and honeycomb structure.

10 This structure is obtained by expanding the clay slips more than their surface tension will permit, thus rupturing the cellular structure. Also using insufficient bonding material to fill the voids in the aggregate tends to form such a structure. A 15 material of this sort has, in general, less structural strength than that shown in Fig. 5 but has higher absorption of sound. Any coating such as 62 which is applied to a sound absorbing material should not be imperforate.

20 The ware may be any size or shape and may be used as part of any building structure. Except for a little calcium sulphate, a trace of sodium sulphate formed in the reaction and a trace of organic matter, the latter representing the 25 soap bark and gum residue, there are usually no foreign materials present in the "green" ware. The burning of the product is, therefore, dependent largely on the characteristics of the original 30 clay used. The final product contains nothing except material of ceramic character.

The details of the process and apparatus may be varied considerably without departing from the spirit of the invention. The above description should therefore be taken as illustrative and 35 not in a limiting sense, the scope of the invention being defined by the appended claims.

The invention claimed is:

1. A process for making cellular ceramic ware including preparing two mutually reactive clay 40 slips, mixing same to form a frothed structure molding into units in which this structure is embodied, drying and burning the ware in frothed condition.

2. A process for forming cellular ceramic ware including mixing a plurality of reactive clay 45 slips with each other at a rate substantially greater than their speed of reaction to form a product which has a frothed structure molding into units in which this structure is embodied, 50 drying and burning the product.

3. A process for forming cellular ceramic ware which includes mixing chemical frothing agents with wet liquid clay, dividing the clay to expose 55 a relatively large surface to an elevated temperature to bring about a reaction molding the

resulting material into units which have a frothed structure, drying and burning the product.

4. A process for forming cellular ceramic ware which includes heating a dried expanded clay material to form an absorbent relatively non-miscible aggregate, coating the aggregate with binding material, depositing the coated and expanded material in a form and allowing to set to form an expanded product, drying and burning the same.

5. A process for forming a cellular ceramic material which comprises forming an acidulated slip, a carbonate-containing slip, mixing the two at a speed substantially greater than their speed of reaction to form a frothed slip and drying in such a manner as to preserve the resulting structure.

6. A process for forming cellular ceramic ware comprising expanding liquid clay, drying and hardening the clay in expanded condition to form a hardened absorbent aggregate, bonding the aggregate with more liquid clay, molding into units, drying and burning.

7. A process for forming cellular ceramic ware which includes forming a plurality of reactive clay slips which contain clay in relatively deflocculated condition, mixing and heating to form a frothed structure employing frothed material thus formed to mold an expanded unit, drying and hardening the product.

8. A process for manufacturing cellular ceramic ware comprising expanding clay in wet liquid condition, drying relatively rapidly in relatively distributed condition, heating to form an absorbent hardened aggregate, bonding with additional liquid clay, molding, drying and burning the product.

9. A process for forming cellular ceramic ware which comprises forming an expanded hardened aggregate of clay, mixing with frothed clay to bond the aggregate to set the froth, molding into units, drying, trimming and burning to form a permanent material.

10. A process for forming cellular ceramic ware which includes forming a frothed clay slip, drying same rapidly to form a cellular aggregate, re-mixing with other clay which burns to a different color, molding into slabs, trimming to expose the expanded structure and burning to form a plurality of colors on the trimmed surface.

11. An apparatus for forming expanded ceramic ware including a plurality of clay-slip feeding devices, a plurality of passages into a mixing device, means for rapid continuous mixing and means for dehydrating the product.

EDWARD R. POWELL.

60 135

65 140

70 145

75 150